

C. S. WICKES,  
METHOD OF MAKING DIAPHRAGMS,  
APPLICATION FILED SEPT. 20, 1912.

1,213,051.

Patented Jan. 16, 1917.

2 SHEETS—SHEET 1.

Fig. 1.



Fig. 2.



Fig. 3.



Fig. 4.



Fig. 5.



Fig. 6.



INVENTOR

Clarence S. Wickes.

A handwritten signature of Clarence S. Wickes.

WITNESSES

W. J. Hartman.

A. G. Brownson.

BY

ATTORNEY

C. S. WICKES,  
METHOD OF MAKING DIAPHRAGMS,  
APPLICATION FILED SEPT. 20, 1912.

1,213,051.

Patented Jan. 16, 1917.

2 SHEETS—SHEET 2.

Fig. 7.



Fig. 9.



Fig. 8.



Fig. 10.



Fig. 11.



Fig. 14.



Fig. 15.



Fig. 13.

Fig. 16.



WITNESSES

F. J. Hartman.  
Alton B. Moulton

BY

Horace Letts.

ATTORNEY

INVENTOR

Clarence S. Wickes.

# UNITED STATES PATENT OFFICE.

CLARENCE S. WICKES, OF MERCHANTVILLE BOROUGH, NEW JERSEY, ASSIGNEE TO  
VICTOR TALKING MACHINE COMPANY, A CORPORATION OF NEW JERSEY.

## METHOD OF MAKING DIAPHRAGMS.

1,213,051.

Specification of Letters Patent. Patented Jan. 16, 1917.

Application filed September 20, 1912. Serial No. 721,415.

To all whom it may concern:

Be it known that I, CLARENCE S. WICKES, a citizen of the United States, and a resident of Merchantville Borough, county of 5 Camden, and State of New Jersey, have invented certain new and useful Improvements in Methods of Making Diaphragms, of which the following is a full, clear, and exact disclosure.

10 My invention relates particularly to diaphragms used in connection with acoustical instruments, such as talking machines, phonographs, gramophones and the like, and to the method of making the same, and 15 the objects of my invention are to produce a diaphragm which is strong, uniformly elastic, durable, homogeneous and which is unaffected by ordinary changes in temperature or humidity; to reduce the cost of diaphragms such as are used in acoustical instruments, and to be able to make a large 20 number of diaphragms having substantially identical and uniform acoustical properties.

A further object of my invention is to 25 produce a diaphragm having the properties and characteristics above indicated, in a simple inexpensive manner, and by the performance of a comparatively few and simple steps.

30 A further object of my invention is to produce, by a molding or pressing process, a diaphragm which, when the process is completed, is substantially implastic and which permanently holds or retains the 35 shape into which it has been formed.

A further object of my invention is to 40 form a diaphragm out of a material which is at first plastic or thermo-plastic, or capable of being molded, or made to flow, and during or substantially immediately after being molded or pressed, changes in physical and chemical properties, into an im- 45 plastic, elastic, insoluble, substantially infusible material, all of these latter properties being desirable in the completed dia- phragm.

A further object of my invention is to 50 produce a diaphragm comprising a thin vibratory portion, unitarily or substantially integrally united to a relatively heavy rim portion of material having similar characteristics to the said vibratory portion, and in which a radial tension may be produced

upon or imparted to said thin vibratory portion.

A further object of my invention is to 55 make a diaphragm having a rigid rim and a central vibratory portion, both composed substantially of final condensation or reaction products of phenol and formaldehyde, 60 but in which the final condensation product of the rim shrinks less or has a less tendency to shrink under ordinary conditions than the final condensation or reaction product of which the thin central or vibratory portion is composed, so that after the diaphragm has been formed, the shrinking of 65 the thin vibratory portion to a greater extent or degree than the rim portion, will stretch or tend to stretch the central portion and will produce, or tend to produce 70 a substantially radial tension upon the thin vibratory portion of the diaphragm.

A further object of my invention is to 75 produce a radial tension in the thin vibratory portion of a diaphragm, by employing the same condensation or reaction product of phenol or formaldehyde in both the rim and vibratory portion, but mixed or used in conjunction with a different filler or body 80 for the vibratory portion of the diaphragm than that used for the rim portion.

Other objects of my invention will appear in the specification and claims below.

Figure 1 is a perspective view of a disk, 85 and a plurality of annuli or rings from which a diaphragm may be made; Figs. 2 and 3 are diametrical sections through the disk and rings when arranged in juxtaposition, the arrangement in Fig. 3 being a 90 slightly different and modified arrangement from that shown in Fig. 2; Fig. 4 is a diametrical section of a die which is adapted to be used in the production of a diaphragm in accordance with this invention; Fig. 5 95 is a diametrical section through a diaphragm, made in such a mold or die as is shown in Fig. 4; Fig. 6 is a plan view of the diaphragm shown in Fig. 5; Figs. 7, 9, 12 and 14 are sectional views through dies 100 or presses arranged to produce diaphragms of different shapes, and Figs. 8, 10, 13 and 15 show the diaphragms produced in the said dies respectively; Fig. 11 is a view of annuli or rings formed from sheets and arranged juxtapose, and upon a disk or plate 105

to be converted and changed into the diaphragm illustrated in Fig. 13 in the die or press shown in Fig. 12, and Fig. 16 is a sectional view of a further modified form of 5 diaphragm.

In setting forth the invention forming the subject-matter of this application, an understanding of the same will probably be more readily had if the process be first described.

In carrying out the process, I first coat or impregnate a sheet of fibrous material, such as fabric, paper, blotting paper, sheets of fibrous pulp, or similar material, with a 15 plastic, semi-plastic or thermo-plastic condensation or reaction product of phenol or its homologues, and formaldehyde or its polymers, with an alkaline base, or some equivalent or similar condensation or reaction product. One condensation product of phenol and formaldehyde, such as I have previously referred to and which readily lends itself to the purpose of this invention, is bakelite. Bakelite is a well known 20 commercial product and may be readily obtained either in solid form or in solution. The said sheet of fibrous material may be so coated or partially impregnated or thoroughly impregnated by immersing the same in a solution of said plastic reaction or condensation product, by painting the said sheet with said condensation or reaction product alone, or dissolved in a suitable solvent, or by flowing a solution of the same over said sheet. 25 Acetone, amyl-acetate, alcohol and other suitable solvents may be used for obtaining a suitable solution of the said plastic or thermo-plastic condensation or reaction product.

40 The sheet of fibrous material so coated or impregnated, is then dried. This coated or impregnated fibrous sheet is plastic or thermo-plastic; that is to say, it is moldable or impressible under the proper degree of 45 heat and pressure, and it will flow within reasonable limits, when subjected to heat and pressure, to conform to a mold. The sheet heretofore described by me may consist of a sheet of ordinary blotting paper coated 50 or impregnated with bakelite or similar condensation product of phenol and formaldehyde. The said coated or impregnated sheet may then be subjected between plates, or in a die, to heat and pressure, preferably to a 55 pressure of substantially 1500 pounds per square inch, at a temperature of substantially 340 degrees F., although it is to be understood that the pressure and temperature may vary when different though similarly 60 acting materials, are employed. As a result of this treatment the coated, partially impregnated or thoroughly impregnated sheet undergoes marked physical and chemical changes. A further and different condensation product is formed from said plastic or

thermo-plastic condensation or reaction product, under the application of heat and pressure, and the fibrous sheet of material becomes, if possible, more thoroughly impregnated with the said further condensation or reaction product of phenol or its homologues, and formaldehyde or its polymers, or of the materials originally used, which final condensation or reaction product is hard, elastic, implastic and unmoldable, 70 glassy and substantially insoluble in any known solution. The sheet so impregnated with the said final condensation or reaction product will be found to be substantially homogeneous throughout, and translucent, if 75 not quite transparent.

Diaphragms for sound boxes for talking machines or other acoustical instruments may be formed from the final sheet so obtained by cutting or punching disks from 80 said sheet, which disks may be mounted in the sound box of talking machines in the same manner that the mica diaphragms are now ordinarily mounted in sound boxes.

Instead of cutting the diaphragms from 90 the sheet after it has been subjected to heat and pressure, the disks may be cut from the sheet which has been coated or impregnated with the plastic or thermo-plastic condensation or reaction product and the disks so 95 formed may be subjected to heat and pressure between dies or plates for the purpose of changing the said disks into disks of the final implastic condensation or reaction product.

In carrying out the process above described, I may readily form diaphragms of any desired shape or configuration, and in the drawings are shown various forms and types of diaphragms produced by the process 105 above indicated and set forth.

After the sheet of fibrous material has been impregnated or coated with the plastic or thermo-plastic condensation or reaction product, and dried, I may cut or stamp 110 from said sheet disks 1 of substantially the size of the desired diaphragm, and I also cut or stamp from said sheet of fibrous material, rings or annuli 2, the outer diameter of which is substantially the same as that of 115 the disks and I place one or more of said annuli on opposite sides of said disk, arranging said disks and annuli concentrically as shown in Fig. 1. So arranged and assembled, as shown in Fig. 2 I place the disks 120 and rings within a mold or die, the surfaces between which are shaped to give the final desired shape to the diaphragm and subject the rings and annuli so placed in the mold to the desired degree of heat and pressure. 125 As a result of this treatment, the plastic or thermo-plastic condensation or reaction product is changed into a further and different condensation or reaction product in the manner above described, and during this 130

change, the material interposed between the two sections of the mold will flow and fill the mold and take the shape given to it by the mold or die, and thus change into a material which will not flow or fuse or further change.

Referring to Fig. 4, when the superimposed rings and annuli shown in Figs. 2 and 3 are placed between the two parts 3 and 4 of the die 5, which parts 3 and 4 are provided with suitable rings or channels 6—6, preferably opposite each other, and subjected to heat and pressure, the various layers which make up the structures shown in Figs. 2 and 3, will be integrally united and will form a single substantially homogeneous unitary diaphragm, such as is shown in Figs. 5 and 6. While being subjected to heat and pressure, the said plastic or thermoplastic condensation or reaction product is changed into a further condensation or reaction product, and while the final product is being formed or just before the final product is formed, the material of the structures shown in Figs. 2 and 3 will flow and fill the space provided within the mold 5.

While such a structure as is shown in Fig. 2 may be treated in such a die as is shown in Fig. 4, to produce the diaphragm 7 shown in Fig. 5, the process may be facilitated and more easily carried out if the exterior diameters of the rings and the interior diameters of the rings 2' be made progressively smaller and larger respectively, so that the structure formed before treatment approximates the final desired form.

By the performance of the steps of the process above described, a diaphragm having a thin relatively flexible elastic non-fusible implastic interior or central portion 8, and an integral unitary hard inflexible rim portion 9, is readily formed from composite or built up structures such as are shown in Figs. 2 and 3.

While I have shown in Figs. 5 and 6 a diaphragm in which the thickened rim or edge 9 is substantially rectangular in cross section, the diagonals of the rectangle of the cross section being arranged normal to the plane of the diaphragm, it is to be understood that I do not limit myself to this particular form or shape. Thus, if it be deemed advisable to produce a diaphragm such as is shown in Fig. 8, the composite structure shown in Fig. 2 may be pressed in such a die as is shown in Fig. 7 and simultaneously heated, or if such a diaphragm as is shown in Fig. 10 is to be produced, a composite structure similar to that shown in Fig. 3 may be placed between the halves of the die shown in Fig. 9 and similarly pressed.

If it is desired to make a diaphragm having an integral flange upon one side thereof only, such as is shown in Fig. 13, a series of narrow rings or annuli cut from the sheet

impregnated with the said plastic or thermoplastic condensation or reaction product are arranged juxtapose and superposed upon the disk 1, to form a limited ring or wall or flange, and then placed within the die shown in Fig. 12, and subjected to heat and pressure. It is further to be understood that when a plain diaphragm similar to the plain mica diaphragms commonly used in the sound boxes for talking machines is to be produced, a plain disk 1 may be placed between the halves of such a die as is shown in Fig. 14, and subjected to heat and pressure, with the result that the plain diaphragm shown in Fig. 15, will be readily produced. As has been indicated above, however, the entire sheet of fibrous material coated, impregnated or partially impregnated with the said plastic or thermoplastic condensation or reaction product may be subjected between plates to the desired pressure and temperature, and the whole sheet changed or transformed into the said implastic condensation or reaction product, and from this said latter sheet finished diaphragms, substantially identical with that shown in Fig. 15, may be cut or punched in any desired way.

The diaphragm shown in Fig. 16 is of the same general type as illustrated in Figs. 5, 8 and 10 above described, except that the thickness of the flexible portion 8, adjacent the rim 9, is reduced, as at 10, in order to make the central portion 8 more flexible, vibratable or yielding, and more readily acted upon by the slight impulses produced by sound waves.

A diaphragm produced by the process above described will be a substantially homogeneous integral structure, notwithstanding the fact that a plurality of layers or thicknesses of material may have been used in making the same, and the rim or flange will be integral with the body or flexible portion thereof. Moreover, the finished diaphragm being impervious to moisture and implastic and infusible, will not be affected by changes in temperature or atmospheric conditions, and will therefore retain the shape into which it has been finally pressed.

It is to be understood that my invention is not to be construed as limited to the exact materials above described or referred to, nor to the exact pressures and temperatures indicated, since the same may vary within reasonable limits, and my invention contemplates the making of diaphragms out of any material which, during the initial stage of its treatment may be shaped or molded, and which, after taking the desired shape, is changed in its chemical and physical properties into substantially implastic material, and I have used the expression "plastic condensation or reaction product of phenol and formaldehyde" to signify broadly any con-

4

densation or reaction product of phenol or its homologues, or any material similar to phenol, with formaldehyde or its polymers, or any material similar to formaldehyde, or 5 any similar plastic condensation or reaction product, which is moldable or impres-  
sible with or without the application of heat or pressure thereto; the expression "thermo-  
plastic" to indicate the property or quality 10 of a material as a result of which the mate-  
rial may be molded or impressed, or made  
to flow when subjected to heat or to heat  
and pressure; and the expression "implastic  
condensation or reaction product of phenol  
15 and formaldehyde" to signify broadly, and  
substantially implastic or unmoldable con-  
densation or reaction product produced by  
a further condensation of the said plastic  
product, preferably by the application  
20 thereto of heat or pressure, or both. It is  
also to be understood that the fibrous mate-  
rial which is originally impregnated or  
coated with the plastic condensation or re-  
action product, acts mainly as a body or  
25 filler, and if it is so desired, may be omitted  
and the original sheets may be formed out  
of the plastic condensation or reaction prod-  
uct alone. In practice, however, I prefer to  
use a body or filler of fibrous material.  
30 Numerous condensation or reaction prod-  
ucts of phenol and its homologues, and for-  
maldehyde or its polymers, or similar ma-  
terials, may be found on the market, and I  
therefore, do not wish to limit myself to  
35 any particular one of them. For illustra-  
tive purposes, however, I might state that  
the condensation product of phenol and for-  
maldehyde, known commercially as bakes-  
lite, is one and among those condensation or  
40 reaction products which may be used by me  
in the diaphragm described above, and the  
method of making the same.

In a diaphragm made in the manner and  
of the material before set forth, with a  
45 difference in the surface area per unit mass  
between the thin vibratory portion and the  
rim portion, there may be a tendency of the  
thin vibratory portion to shrink slightly,  
and to a greater degree than the heavy  
50 thicker unitary substantially integral edge  
or rim, and the degree or extent to which  
one of the said two parts may shrink with  
respect to the other may be greatly modified  
or affected by the use of different amounts  
55 or proportions of the vegetable, animal, or  
mineral fiber used with the different plastic  
or thermo-plastic condensation or reaction  
products. In other words, the amount of  
shrinkage in a finished diaphragm may be  
60 made to depend a great deal upon the par-  
ticular filler and the particular plastic or  
thermo-plastic condensation or reaction  
product and the particular proportions of  
each employed.

65 Certain proportions of one to the other

will produce a structure in which there is  
substantially no shrinkage, whereas certain  
other proportions of these materials will  
result in a product which may shrink or  
tend to shrink quite a deal. Therefore, by 70  
making the thinner vibratory portion of a  
composition containing one particular filler  
with a certain amount of the plastic or  
thermo-plastic or other condensation or re-  
action product, and by making the thick 75  
or heavy rim of another filler with the same  
or other proportions of the same or other  
plastic or thermo-plastic condensation or  
reaction products, the amount of shrinkage  
in or the tendency to shrink of the said thin 80  
vibratory portion, may be greater than that  
of the heavier rim, and this difference in  
shrinkage of the two parts of the dia-  
phragm, or the tendency of one to shrink  
to a greater extent than the other may be 85  
made to produce a radial tension or stretch  
of the thin vibratory portion when such ten-  
sion is desired. If, on the other hand, how-  
ever, it be desirable to impart or impose  
substantially no such tension upon the thin 90  
vibratory portion, different materials or  
different proportions of the above indicated  
ingredients may be employed for the vi-  
bratory portion and for the rim, so that the  
shrinkage of both of the said parts of the 95  
finished diaphragm will be the same, or so  
that there will be no relative shrinkage of  
either of said parts with regard to the other.

This shrinking of the diaphragm may in  
some cases, be effected or modified by an 100  
aging of the same, but after the finished  
diaphragm has assumed its final condition,  
the composition will remain substantially  
stable and the finished product will be un-  
affected by heat, moisture or other atmos-  
pheric changes or conditions. The dia- 105  
phragms so made will not warp nor twist  
in their final form, which characteristic is  
also desirable in this kind of a structure.

The diaphragms above described possess 110  
qualities which make them particularly  
adapted for the sound boxes for sound re-  
producing machines and for other acous-  
tical instruments. Thus, the low specific  
115 gravity of the condensation products above  
referred to (about 1.25) as compared with  
that of glass, mica, or the metals, gives them  
a small vibrating inertia. Their resiliency  
is of a peculiar nature, very different from  
the elasticity of rubber, and it is of that  
type which makes them particularly well  
suited for the reproduction of sound. The  
facility with which various fibrous sub-  
stances or other suitable materials may be  
120 incorporated into the structure of the dia-  
phragm permits of a predetermined varia-  
tion in specific gravity, vibrating inertia,  
texture and general and chemical and acous-  
tical properties. A further quality or char-  
acteristic of the said diaphragms resides in 125  
130

the fact that the same are not substantially altered in shape or substance by hydrolysis or other chemical action induced by atmospheric conditions, and that they are substantially unaffected by high and low temperatures.

It is further to be observed that the great uniformity in the product may be comparatively easily obtained, a result not attained when mica, glass, rubber, or the metals are used for the diaphragms, while the relative cheapness of the materials employed and the simplicity of the process very materially reduce the cost of the completed diaphragm.

10 While broadly my invention is independent of any particular form or shape of diaphragm, the preferred form embodies in its construction a relatively heavy rigid and strong rim or edge, as indicated in Figs. 5, 8, 10, 13 and 16, as such a rim or edge tends to make the entire structure stiff or self supporting, and to hold the flexible or vibratable portion 8 taut or in a fixed plane, and further tends to overcome or offset any 15 tendency of the diaphragm as a whole to warp, or become distorted. As has been above set forth, shrinkage of the finished diaphragm or the tendency to shrink, or change in its size, can be greatly modified 20 and, if desired, substantially overcome by the use of the proper amount or proportion of vegetable, animal or mineral fiber or filler with the particular plastic or thermo-plastic condensation or reaction product employed.

25 In other words, the amount of shrinkage in a finished diaphragm will depend substantially upon the particular filler, and the particular plastic or thermo-plastic condensation or reaction product, and the particular proportions of the same which are employed, and certain proportions of one to the other are found to result in a structure in which the shrinkage is very small or practically nothing. These 30 properties or qualities, therefore, enable one to construct a substantially uniform homogeneous integral diaphragm in which the central or vibratory portion may be made to have substantially no radial tension, or, if 35 so desired, may be made to have a substantially predetermined radial tension imparted thereto.

Having thus described my invention, what I claim and desire to protect by Letters Patent of the United States is:

1. The method of making a diaphragm for acoustical instruments which consists in impregnating a sheet of fibrous material with a thermo-plastic condensation product of phenol and formaldehyde in solution, forming a disk from the same, superposing upon the edge portion of said disk an annulus of similarly impregnated sheet material, subjecting said disk and annulus to heat and pressure to change said condensation

product into a further condensation product and to form thereby an integral homogeneous infusible implastic diaphragm, having a stiffening rim.

2. The method of making a diaphragm for acoustical instruments which consists in impregnating a sheet of fibrous material with a thermo-plastic condensation product of phenol and formaldehyde in solution, forming a disk from the same, superposing upon the edge portion of said disk an annulus of similarly impregnated sheet material, subjecting said disk and annulus to heat and pressure in a mold to further condense said condensation product, and to form thereby an integral homogeneous infusible implastic diaphragm having a stiff substantially integral rim.

3. The method of making a diaphragm for acoustical instruments which consists in impregnating a sheet of fibrous material with a condensation or reaction product of phenol and formaldehyde, forming a disk from the same, superposing upon the edge portion of said disk a plurality of annuli formed from sheets of material similarly impregnated and subjecting said disk and annuli to heat and pressure to further condense said condensation or reaction product and to form thereby an integral homogeneous infusible implastic diaphragm having a stiff substantially integral rim.

4. The method of making a diaphragm for acoustical instruments which consists in impregnating a sheet of fibrous material with a condensation or reaction product of phenol and formaldehyde, forming a disk from the same, superposing upon the edge portion of said disk a plurality of annuli formed from sheets of material similarly impregnated, and subjecting said disk and annuli to heat and pressure in a mold to further condense said condensation product and to form thereby an integral homogeneous infusible implastic diaphragm having a stiffening rim at the edge thereof.

5. The method of forming a diaphragm for acoustical instruments which consists in impregnating a sheet of fibrous material with a thermo-plastic condensation or reaction product of phenol and formaldehyde, forming a disk from the same, placing upon the opposite faces of said disk and adjacent the edges of the same, a plurality of superposed annuli formed from sheet material similarly impregnated, subjecting said disk and annuli to heat and pressure in a mold conforming generally to the form of said superposed disk and annuli to change the form of said material to that of the mold and to change said condensation product into an implastic product, thereby to form an integral homogeneous infusible implastic diaphragm, having a stiff substantially integral rim.

6. The method of forming a diaphragm for acoustical instruments which consists in impregnating a sheet of fibrous material with a plastic condensation or reaction product of phenol and formaldehyde, forming a disk from the same, placing upon opposite faces of said disk and adjacent the edges of the same, a plurality of superposed annuli formed from sheets of material similarly impregnated to approximate the final form of diaphragm desired, subjecting said disk and annuli to heat and pressure in a mold and thereby changing said plastic condensation or reaction product into an im- 10 plastic condensation or reaction product of phenol and formaldehyde, distributed sub-stantially homogeneously throughout the diaphragm so formed.
7. A method of forming a diaphragm for acoustical instruments, which consists in forming a disk composed substantially of a condensation or reaction product of phenol and formaldehyde, superposing upon the peripheral portion of said disk an annulus 15 composed substantially of a condensation or reaction product of phenol and formalde-hyde, and subjecting said disk and annulus to heat and pressure to simultaneously change said condensation product into a fur- 20 ther condensation or reaction product and to substantially integrally unite said annulus and disk.
8. A method of forming a diaphragm for acoustical instruments, which consists in forming a disk composed substantially of a condensation or reaction product of phenol and formaldehyde, superposing upon the peripheral portion of said disk an annulus 25 composed of a condensation or reaction product of phenol and formaldehyde, sub-jecting said disk and annulus to heat and pressure to simultaneously change said condensation product into a further condensation or reaction product and substantially 30 integrally unite said disk and annulus, and aging the product so formed.
9. A method of forming a diaphragm for acoustical instruments, which consists in forming a disk composed substantially of a condensation or reaction product of phenol and formaldehyde and a filler, superposing 35 upon the peripheral portion of said disk an annulus of a material composed of a con- densation or reaction product of phenol and formaldehyde and a filler, the proportions 40 of said condensation product and formalde-hyde to the filler in said disk being different from that proportion of said materials in said annulus, subjecting said disk and annulus to heat and pressure to change the con- densation product of said disk and annulus 45 into further condensation or reaction products, and to simultaneously integrally unite said annulus and disk.
10. A method of forming a diaphragm for acoustical instruments, which consists in forming a disk composed substantially of a condensation or reaction product of phenol and formaldehyde and a filler, superposing upon the peripheral portion of said disk an annulus of material composed of a con- densation or reaction product of phenol and formaldehyde and a filler, and subjecting 55 said disk and annulus to heat and pressure to simultaneously change said condensation products into further condensation or reaction products, and to substantially integrally unite said disk and annulus, the final condensation or reaction product of said disk having a greater tendency to shrink 60 than the final condensation or reaction product of said rim.
11. A method of forming a diaphragm for acoustical instruments, which consists in forming a disk composed substantially of a condensation or reaction product of phenol and formaldehyde and a filler, superposing upon the peripheral portion of said disk an annulus of material composed of a con- densation or reaction product of phenol and formaldehyde and a filler, and subjecting 65 said disk and annulus to heat and pressure to simultaneously change said condensation products into further condensation or reaction products, and to substantially integrally unite said disk and annulus, the final condensation or reaction product of said rim having a tendency to shrink.
- In witness whereof, I have hereunto set my hand this 18th day of September, 1912.
- CLARENCE S. WICKES.
- Witnesses:
- FRANK B. MIDDLETON, Jr.,  
CHARLES F. WILLARD.